

## UNITED STATES PATENT OFFICE.

ALBERT BODMER, OF WATTWIL, SWITZERLAND, ASSIGNOR TO HEBERLEIN & CO. A. G.,  
OF WATTWIL, SWITZERLAND, A CORPORATION OF SWITZERLAND.

## TREATING COTTON FIBERS TO PRODUCE WOOLLIKE EFFECTS.

No Drawing. Application filed September 8, 1926, Serial No. 134,332, and in Germany September 16, 1925.

My invention relates to process of treating cotton goods, and more particularly the invention relates to a process of producing cotton goods with a wool-like finish.

It is well known that cotton may be treated with (concentrated) nitric acid to thereby produce a good permanent finish wool-like effect resembling wool in looks, feel and in caloric quality. This treatment as is now well known in the art, may be produced with or without a preliminary mercerization treatment. As an example of a treatment of cotton goods by nitric acid to produce a wool-like effect, reference is made to United States Letters Patent, No. 1,439,515, to Georges Heberlein, patented December 19, 1922, wherein such a process is described and claimed.

However, when cotton is processed with nitric acid to produce said permanent finish wool effect, certain properties are attendant in the resultant product which are highly undesirable in textile materials. For example, vegetable fibrous material, such as cotton, which has been modified in this manner, possesses a yellowish color, and it also has a very great affinity for dyes and consequently the uniform coloring of such a product is extremely difficult. In addition, these products are very sensitive to alkali, so much so that even a washing with soda is attended with injury to the fibers, so that when one cannot bleach the goods to remove the yellow color without damage to the goods. Dyeing with vat dyes in an alkali bath likewise brings about a weakening of the material.

The object of this invention is to improve such nitrated permanent finish textile materials, by overcoming these objectionable characteristics.

The invention comprises the improved product and also the process of producing same. The invention will be more readily understood from the following description including one or more examples of how the product may be produced; and the invention will be more fully set forth in the appended claims.

Upon making investigations, I have observed that small quantities of nitrogen are always absorbed and retained by the fibers in the treatment of the cotton with nitric acid. And I have discovered that if the fibers that

have been thus treated are denitrated, the surprising fact becomes manifest, that the affinity for dyes has reverted to a normal amount and that at the same time the sensitiveness to alkali has disappeared. Besides this, a more extensive modification in the structure of the fiber has taken place which manifests itself in a considerable heightening of the wool effect. By this invention it is now easily possible to produce uniform colorings, even by means of vat dyes. Even alkaline boilings are no longer capable of detrimentally affecting the wool-like finish so that it is now possible to eliminate, by means of supplementary bleaching, the yellowish tone that has been caused by the treatment with nitric acid, and to obtain a perfectly white fiber. The resistance to alkali that is attained also results in greatly increasing the fastness as to color; and the permanence of textiles that have been improved in this manner.

While nitrated cotton wool effects, i. e., those produced by treatment with nitric acid, have been very excellent as to their wool qualities, yet the above-mentioned detrimental characteristics have been such as to greatly curb an extensive commercial use of the same; but by the simple treatment according to this invention, not only have all of these objections been overcome, but the wool effect itself is actually improved.

This denitration may be carried out in any suitable manner. For example, I have found it to be satisfactory to denitrate in a manner similar to the method used in the production of artificial silk from cellulose nitrate; and furthermore, the denitrating agents that are in use or are suitable for use in the production of artificial silk from cellulose nitrate are likewise satisfactory in connection with my invention. Thus by way of example, there are found to be satisfactory, especially the sulfides and sulfohydrates of the alkalis, alkaline earths and ammonium, in which connection these agents may be used singly or mixed one with another. Also the salts of the low stages of oxidation of multivalent metals may be employed for this purpose with more or less extensive effect in a weakly acid or ammoniacal solution, for example cuprous chloride, ferrous chloride, stannous chloride, and others.

While any suitable denitrating treatment

may be used, I give by way of example only, the following treatments that have been found to give satisfactory results:

5 *Example No. 1.*

Vegetable fabrics after previous desizing and washing, preferably unbleached are mercerized without tension with NaOH of about 30° Bé. at room temperature for 5 minutes, 10 and are washed out, soured, washed and dried. Goods thus pretreated are exposed to the action of nitric acid with an acid content of about 72% for about 8 minutes, and are washed out in a denitrating bath. This 15 denitrating bath may consist of a 5% solution of NaSH and goods may remain in the bath at room temperature for instance for 30 to 60 minutes, then bleached and dyed.

20 *Example No. 2.*

Raw cotton yarn is washed out and dried, and immersed in a solution of about 74% HNO<sub>3</sub> content for a period of about 5 minutes. When sufficiently acted upon the acid 25 is washed out and the yarn denitrated in a cold bath containing about 2% NH<sub>4</sub>SH for about 30 minutes. It is then washed out and prepared for bleaching and dyeing in the customary manner.

30 As will be obvious to those skilled in the art, after understanding my invention, the invention is not to be limited to the treatment of cotton fabrics, for the invention is also

applicable to the treatment of yarns and threads made of cotton fiber, and by the term "goods" I wish to be understood as including 35 cotton fabrics and yarns; nor to any particular denitrating treatment; and while the denitration is especially useful in connection with nitrated wool effects on cotton fibers, 40 it may also be useful in connection with other nitrated effects on cotton goods having some of the foregoing objections.

Having thus described my invention, what I claim as new and desire to secure by Letters 45 Patent, is:

1. Method of treating cotton goods which comprises producing thereon a permanent finish wool-like effect by treating the goods with nitric acid, denitrating the goods to 50 render them less sensitive to alkali prior to any finishing treatment involving alkali, and subsequently treating the goods with an alkali substance to further finish the same.

2. Method of treating cotton goods which 55 comprises producing thereon a permanent finish wool-like effect by treating the goods with nitric acid, reducing the affinity of the goods for dyes and increasing the fastness of the color by denitrating the goods, prior 60 to any dyeing or other treatment involving an alkali, and subsequently dyeing the goods with a dye containing alkali.

In testimony whereof I have signed my name to this specification.

ALBERT BODMER.